

## UNITED STATES PATENT OFFICE.

FRANK FISHER, OF BROOKLYN, NEW YORK.

## INK-REDUCER AND PROCESS OF MAKING SAME.

SPECIFICATION forming part of Letters Patent No. 730,897, dated June 16, 1903.

Application filed October 23, 1902. Serial No. 128,424. (No specimens.)

*To all whom it may concern:*

Be it known that I, FRANK FISHER, a citizen of the United States, and a resident of the city of New York, borough of Brooklyn, in the county of Kings and State of New York, have invented a new and Improved Ink-Reducer and Process of Making the Same, of which the following is a full, clear, and exact description.

10 This invention relates to a means for reducing ink, whereby the ink is placed in a condition facilitating its proper manipulation and application to the paper.

By means of my invention the ink is softened and caused to properly adhere to the paper, thus preventing the ink from peeling off of the paper. The reducer also prevents the ink from being offset from the paper—that is to say, it prevents the application of 15 excessive quantities of ink. Owing to this and to the fact that the ink treated with the reducer dries very rapidly, the fresh-printed sheets, placed one upon the other, will not adhere nor will a lower sheet transmit its 20 impression to the back of an upper sheet.

To this end the invention consists in a reducer composed of certain ingredients, to be hereinafter specified, and also in a novel process of combining these ingredients to produce 25 the proper result.

The ingredients of my improved ink-reducer consist, in varnish, one and one-third quarts; balsam of copaiba, one and one-third quarts; Japan drier, one gill; sweet-oil, (preferably French,) one and one-third quarts; citron-oil, one gill.

The varnish serves to soften or render the ink more liquid, at the same time retaining the body thereof. The balsam of copaiba produces luster in the ink and causes it to permeate the very fabric of the paper. The Japan drier is used to cause the ink to set immedi-

ately, thus preventing it from blurring. The sweet-oil is used to give the ink a uniform consistency and to prevent it from adhering 45 to other surfaces after being applied to the paper, which adherence would result in the peeling of the ink from the surface to which it was at first and intentionally applied. The citron-oil is used to disguise the odor of the 50 varnish.

In the process of producing the improved ink-reducer the sweet-oil is heated, and this heated oil, together with the varnish and balsam of copaiba, is run into and through a 55 filter. To this filtered mixture the citron-oil and the Japan drier are added, producing the finished product.

The ink-reducer is used by mixing it with the ink either prior to the application of the 60 ink to the font in the printing-press or by pouring the reducer into the font in which the ink has already been placed.

Having thus described my invention, I claim as new and desire to secure by Letters 65 Patent—

" 1. An improved ink-reducer, consisting of varnish, balsam of copaiba, Japan drier, sweet-oil, and citron-oil in essentially the proportions stated.

2. The process of producing the herein-described ink-reducer, such process consisting first in heating the sweet-oil, second in simultaneously admixing and filtering the sweet-oil, varnish and balsam of copaiba, and third, 75 in adding the citron-oil and Japan drier to the aforesaid filtered mixture.

In testimony whereof I have signed my name to this specification in the presence of two subscribing witnesses.

FRANK FISHER.

Witnesses:

SEAMAN E. DENTON,  
THOMAS I. FURLONG.